

## UNITED STATES PATENT OFFICE

2,608,460

REDUCTION OF THE SWELLING INDEX OF  
REGENERATED CELLULOSE FIBERS BY  
STEAM UNDER PRESSURENicolas Drisch and André Bonnet, Paris, France,  
assignors to Comptoir des Textiles Artificiels, a  
corporation of FranceNo Drawing. Application February 15, 1951, Se-  
rial No. 211,195. In France April 21, 1944

## 2 Claims. (Cl. 8—130.1)

1

This invention relates to a new and improved process of treating absorbent textile fibers and to the product resulting therefrom. More particularly, it relates to substantially reducing the hygroscopicity of regenerated cellulose staple fibers and the product resulting therefrom.

This application is a continuation-in-part of our co-pending application for Process of Treating Absorbent Textiles, Serial No. 723,902, filed January 23, 1947 now abandoned.

Hygroscopicity is herein defined as the index of swelling and is determined as follows: The cellulose material, after being saturated with water, as by dipping in water, is centrifuged for 10 minutes in a centrifugal drier 30 centimeters in diameter and rotating at 3000 R. P. M. The index of swelling is the weight of the water retained by the centrifuged material compared with the original dry material.

U. S. Patent No. 1,544,835 to Brandenberger discloses a process of reducing the hygroscopicity of cellulose hydrates, and particularly regenerated cellulose, by subjecting such material in its dry state to the action of dry saturated steam, preferably under pressure, in a closed vessel. Such a process will reduce the swelling index of regenerated cellulose having a swelling index of between 80% and 150% to 50% or below.

In addition to the reduction in hygroscopicity, the treated product acquired other beneficial results. The shrinkage determined by the decrease in the dimensions resulting from washing with water, followed by drying without tension, of the steam-treated cellulose materials, such as pellicles, fibers, threads or fabrics made therefrom, was materially lower than that which characterized the untreated cellulose material.

However, the process of the Brandenberger Patent No. 1,544,835 possessed a serious disadvantage in that the cellulose subjected to the process underwent a depolymerization which was manifest as a deterioration in the mechanical properties and which produced a yellowing of the product.

An object of this invention is to provide a method of substantially reducing the swelling index of regenerated cellulose staple fibers without any appreciable depolymerization of the cellulose.

A further object of the invention is to provide a method of treating regenerated cellulose textile materials to materially reduce their swelling index without affecting their serimetric properties.

Other and additional objects will become apparent hereinafter.

2

We have found that the depolymerization is due to the wetting of the fibers in the mass by condensation of the steam which occurs because the fibers in the mass are initially cold and the inside of the mass remains cold while the steam penetrates slowly due to the pressure of the air within the mass. The fibers which are thus wet are only heated by the steam without coming into direct contact with the steam. Such heating while wet causes depolymerization and forms grayish brown particles indicating non-uniformity of treatment.

This is avoided in accordance with the present invention by means of a two-stage steam treatment in which the mass of fibers is placed in a closed vessel which is evacuated to remove any air or gases from the interior of the mass which would interfere with the free passage of the steam thereto. Dry saturated steam is thus introduced into the vessel until the interior is brought up to the steam pressure. Since the steam penetrates rapidly the entire mass is brought up to treating temperature before substantial condensation can occur. However, in order to remove even this small amount of condensation the steam is again shut off, the vessel evacuated, and the operation repeated. Since the mass is then heated, no condensation occurs. The steam treatment under pressure then continues for a predetermined period after which the steam is shut off and the vessel opened to remove the treated fibers.

The details and manner of practicing the invention will become apparent by reference to the following specific example, it being understood that this example is merely illustrative of an embodiment of the invention and that the scope of the invention is not restricted thereto.

*Example*

One or more 200 pound bales of staple fibers of regenerated cellulose obtained by either the viscose or cuprammonium processes is placed in a large autoclave or is formed into a ball which is placed in such autoclave. After closing the autoclave it is subjected to vacuum of from 5 centimeters to 10 centimeters of mercury. Dry saturated steam of a pressure of from 1.8 to 2 kg. per square centimeter is then introduced until the pressure in the autoclave is brought up to the steam pressure. The steaming is continued a few minutes to bring the entire mass up to the steam temperature. The steam is then shut off and the autoclave again evacuated as before to from 5 to 10 centimeters of mercury to remove all of the moisture from the fibers, after which the steam is again introduced and

the pressure brought up to the steam pressure. This steam treatment is continued for from 2 to 2½ hours, after which the steam is shut off and the autoclave opened.

The following table shows the degree of polymerization and index of swelling of the staple fibers before and after treatment:

|                       | Degree of Polymerization | Swelling Index |
|-----------------------|--------------------------|----------------|
| Untreated fibers..... | 320                      | 105            |
| Treated fibers.....   | 320                      | 58             |

The process is carried out with dry saturated steam under a pressure which may vary between 1.5 and 15 kg. per square centimeter and at the corresponding temperature. In general, a higher pressure requires a shorter treatment and a lower pressure requires a longer treatment. For example, when a pressure of 14 kg. per square centimeter is utilized, a treatment of several minutes is sufficient while with a pressure of 1 kg. per square centimeter a treatment of approximately 4 hours is necessary. In the preferred embodiment pressures of from 1.8 to 2.0 kg. per square centimeter for a period of 2½ to 2 hours are employed.

The process reduces the swelling index, and hence the absorptive power of regenerated cellulose textile materials, without changing the degree of polymerization of the original cellulose. As a result, the serimetric properties of the textiles are not diminished in the least. In certain cases, the tenacity of regenerated cellulose rayon yarn is slightly reduced. However, such slight reduction in tenacity is compensated by an increase in elongation. This increase in elongation is due simply to the shrinkage produced in the course of the treatment and is not due to any deterioration of the cellulose material. The

process additionally results in a product having improved (low) shrinkage and a yellowing considerably less than that of the prior art.

Since it is obvious that various changes and modifications may be made in the above description without departing from the nature or spirit thereof, this invention is not restricted thereto except as set forth in the appended claims.

What is claimed is:

1. A method of materially reducing the hygroscopicity of regenerated cellulose staple fibers without substantially changing their degree of polymerization, which comprises disposing a bale of said fibers in a closed vessel, evacuating the atmosphere in said vessel, then from an outside source introducing dry saturated steam under a pressure of from 1.5 to 15 kg. per sq. cm. into said vessel until the interior of said vessel is brought up to the steam pressure and the mass
- 15 is heated throughout, then shutting off the steam and again evacuating the interior of said vessel, again introducing said steam into said vessel to bring the interior of said vessel up to steam pressure of the entering steam and maintaining said steam pressure in said vessel for a period of a few minutes to four hours, the time varying inversely as the pressure.
- 20 2. The method as claimed in claim 1 wherein the evacuation is carried to between 5 centimeters and 10 centimeters of mercury.

NICOLAS DRISCH.  
ANDRÉ BONNET.

REFERENCES CITED

- 35 35. The following references are of record in the file of this patent:

UNITED STATES PATENTS

- | Number       | Name          | Date         |
|--------------|---------------|--------------|
| 40 1,544,885 | Brandenberger | July 7, 1925 |
| 2,119,261    | Andrews       | May 31, 1938 |